

April 29, 1952

E. R. POWELL

2,594,799

METHOD AND APPARATUS FOR THE MANUFACTURE OF MINERAL WOOL

Filed July 18, 1946



INVENTOR  
EDWARD R. POWELL  
BY *Virgil P. Kline*  
ATTORNEY

Patented Apr. 29, 1952

2,594,799

# UNITED STATES PATENT OFFICE

2,594,799

## METHOD AND APPARATUS FOR THE MANUFACTURE OF MINERAL WOOL

Edward R. Powell, North Plainfield, N. J., assignor to Johns-Manville Corporation, New York, N. Y., a corporation of New York

Application July 18, 1946, Serial No. 684,466

10 Claims. (Cl. 18—2.6)

1

The instant invention relates to the formation of artificial fibers of the types of which glass wool, slag wool, rock wool and the like are the principal commercial examples. More particularly the invention is concerned with an economical method and apparatus which will produce a stronger fiber than heretofore and provide a better control of fiber size.

Prior to the instant invention the methods of converting a raw material, such as glass, slag, rock and other fusible raw materials into fiber form, have been of two sharply different types. The first involves individual formation of a fiber from a single source of liquid material. This method is employed principally in the production of fibers of glass and like materials where the fibers or filaments are drawn from individual orifices of a furnace or other source of molten material. Even though, as is often the case, there may be from 60-200 orifices in the orifice plate of the melting furnace, the process is expensive due to the still relatively low production rate. The process, however, does have the advantage that the fiber size may be accurately controlled and uniform fibers produced.

The second method is directed to multiple fiber formation involving the disintegration of a molten stream of the raw material simultaneously into several thousand fibers. In a conventional method of this kind the molten stream is subjected to the action of a steam blast which shreds the stream into minute droplets which are drawn out into fiber form by the force of the blast. In another method the stream is projected onto the peripheral surface of one or more rotors rotating at high speed, the rotors serving to break up the stream into droplets and to draw them into fibrous form. The multiple formation methods are relatively economical but the fiber does not have many of the desirable properties exhibited by the drawn fibers and the fiber size cannot be readily controlled.

The principal object of the instant invention is the provision of a method, and of an apparatus for carrying out the method, which will have the advantages of both methods of the prior types, but without the disadvantages of either.

Another object of the invention is the provision of such method which permits the use of selected compositions of the raw material not previously usable in multiple fiber production operations. There is a sharp contrast in the fluidities of the melts which have been employed in the two types of procedures described above; for example, in the method involving the drawing of individual fibers, the glass compositions employed for the most part are those which do not become a mobile fluid at the temperatures at which their ingredients begin to volatilize. These melts, such for example as molten plate glass at a tempera-

2

ture of from 2400-2600° F., therefore have a well defined fluidity which will cause them, under controlled conditions, to flow for example 1/2", before solidifying. The melts employed in multiple fiber formation by the use of a steam blast or high speed rotors, may flow from 8-12" under the same conditions. The more viscous melts as employed in individual fiber production processes produce a tough fiber under definite tension, the toughness being due to molecular orientation or to other causes. The fibers obtained by the multiple fiber production system, on the other hand, are relatively weak and irregular.

Another object of the invention is the provision of a method of the multiple fiber production type which may be successfully used with the more viscous melts of the kind previously employed only for drawn fibers.

The multiple formation methods, while commercially practicable with the more fluid melts, have not produced the desired high proportion of fine fibers, due to the fact that the separation or division of the molten stream into molten particles or bodies from which the fibers are drawn is not uniform or definitely controllable. As a result the bodies are of different and relatively uncontrolled size, and produce fibers of a wide range of diameters. It has not been unusual for such methods to produce fibers from 1 1/2-15 microns in diameter and with 30-70% of shot or unfiberized material. This is due specifically to the fact that it has been necessary to spray the original large stream into several thousand droplets or incipient fibers, either by the use of the steam blast or the rotors, and then stretch the droplets or incipient fibers. Only a part of even the more fluid melts separate into the proper droplet size for fine fiber formation. Since coarse fibers made of any of the known inorganic compositions are irritating to the skin and are more or less brittle, the control of the fiber size is of primary importance. Where attempts have been made to use the more viscous melts, it has been found impossible to obtain either uniformity of the droplets or the conversion of any large portion of the stream into droplets of the right size. Accordingly, a further object of the invention is the provision of a method and apparatus which will insure proper control of the droplet size from which the fibers are individually drawn.

A still further object of the invention is the provision of a method and apparatus for the preparation of the molten material to be converted into fibers by a spinning process involving one or, suitably, a plurality of rotors rotating at high speed. The rotors may be generally of the type and driven at the speed of those shown and described, for example, in my copending applications, S. N. 446,067, filed November 18, 1942, now Patent No. 2,399,383, S. N. 486,009, filed

April 29, 1943, now Patent No. 2,428,810, and S. N. 555,359, filed September 22, 1944, now Patent No. 2,520,168. Mechanical examination of the fibers heretofore formed by processes in which a molten stream of raw material is permitted to fall directly on one of the rotors, and is sprayed therefrom onto adjacent rotors, as described in my said co-pending applications, reveals that fiber of 1½-2 microns diameter is formed from particles of 100-200 mesh size, as determined by standard testing sieves. This relationship between particle and fiber size may readily be checked. It can be assumed that the fibers will be about a foot in length since the rotors involved in the process are roughly 1 foot in diameter, and can be expected to make fiber of a length approximately equal to their diameters. That is, the fiber, when drawn to such length, is carried into contact with the rotor and broken off. It may be easily shown that a particle of the size referred to above contains enough material to form a foot of fiber within the 1½-2 micron range, assuming a fair percentage of fiberization. Control of the particle size as provided by the instant invention therefore permits the rotor process of fiberization to become definite and controllable, at least to the right order of magnitude of the fibers.

My invention will be more fully understood and further objects and advantages thereof will become apparent when reference is made to the more detailed description of a preferred embodiment of the invention which is to follow and to the accompanying drawing in which:

Fig. 1 is a diagrammatic, sectional view of an apparatus embodying the instant invention and suitable for carrying out the method thereof; and,

Fig. 2 is a sectional view taken on the line 2—2 of Fig. 1 and looking in the direction indicated by the arrows.

Referring now to the drawings, an air-heating furnace is shown at 10, the furnace including a combustion chamber 12 and a heat transfer chamber 14. The transfer chamber 14 is traversed by a plurality of tubes 16 opening at one end into the combustion chamber 12 through a header 18, and at the other end into a stack 20 through a rear wall 22. Combustion chamber 12 includes a fuel burner 24 which may be of any conventional type and adapted to consume any suitable fuel. For example, the burner may use coal, oil or gas, as desired.

A blower 26 is mounted, preferably above the furnace as shown, to have its discharge side in communication with an air entry port 28 leading into the rear of the transfer chamber 14. Chamber 14 is provided with baffle walls 30 positioned intermediate the front and rear walls of the chamber and extending alternately from its top and bottom walls toward but short of the opposite wall to require air entering port 28 to make a plurality of passes around tubes 16 before it is discharged through a discharge port 32. In the construction shown two baffles are employed to obtain three passes of air around the tubes, but it will be understood that additional baffles may be employed to increase the number of passes where desired.

The air heater described above is of generally conventional type and may be purchased commercially. It may be made of any suitable refractory materials, for example, refractories such as sillimanite or mullite. The tubes 16 may be of a highly heat-resistant material such as a high

grade silicon carbide refractory of the type sold under the name "Carbofrax."

In accordance with the instant invention, stack 20 includes a hopper bottom 34 (see particularly Fig. 2) in communication through a tubular passageway 36 with a material discharge port 38 opening into a furnace 50. Adjacent the upper end of stack 20, or at least at a point remote from the hopper bottom of the stack, is a supply device indicated generally at 40 for feeding a granulated furnace to the stack where it falls, counter-current to the flow of gases exhausted through the stack, to the hopper bottom 34. Device 40 includes a hopper 42 having a bottom orifice in communication with a duct 44 which, in turn, penetrates the wall of the stack. Within duct 44 is a screw feed 46 rotated by any suitable means (not shown) and preferably at a controlled rate to carry the material from the hopper and into the stack. Located in the hopper bottom is a similar screw feed 48 extending into tubular passageway 36 to deliver material from the hopper bottom to the material discharge port 38. The latter screw is made of an alloy steel or non-ferrous alloy which will withstand a high temperature such as 2000° F.

Below air heater 10 is a furnace 50 having, preferably, a dome section 52, cylindrical section 54, and a flattened, generally conical section 56, although the shape of the furnace is not critical and may be varied in a number of particulars, the necessary features being made evident as the description proceeds. The furnace is made of refractory material, similarly as air heater 10. The furnace is in communication with the port 32 of air heater 10 through passage 58 leading into the cylindrical section of the furnace. A burner 60 is located, preferably centrally of dome section 52, the burner utilizing fluid or powdered fuel, similarly as burner 24.

The mouth 62 of the furnace is positioned above the peripheral faces of, preferably, a pair of rotors 64. These rotors, which may be, say, 12" in diameter are made of, or at least include rims or tires of, a heat-resistant steel. The rotors are carried by shafts 65 mounted in planes at an angle to the horizontal, as shown. Shafts 65 are driven by suitable means (not shown) to cause movements of the upper peripheral surfaces of the rotors, preferably towards each other.

In the operation of the apparatus described above, burner 24 is regulated to raise the temperature in combustion chamber 12 to, say, from 2700-2800° F., the flames from the burner being directed by wall 18 into tubes 16. The burnt gases pass from the tubes into stack 20 where they raise the temperature to, say, 2000° F. and are discharged to the atmosphere through the top of the stack. Blower 26 is operated to cause a flow of air through the air heater at a relatively low velocity so that it will be heated to, say, 1600-2000° F. when it reaches exit port 32. As stated above, the construction illustrated provides for three passes of the air around tubes 16 but conditions may require a greater number of baffles to increase the number of passes in order to bring the air to the required temperature. The heated air flows through passage 58 into furnace 50.

Burner 60 is regulated to raise the temperature in furnace 50 above the melting temperature of the raw material, say, a temperature of about 3500° F. for most conventional raw materials.

The selected raw materials previously prepared in granulated form by conventional crushing and

air separation operations to have a predetermined, relatively definite particle size determined by the diameter of the fibers to be produced but, say, of 100-200 mesh, is supplied to hopper 42 and transferred from the hopper at a controlled rate by screw conveyor 46, and discharged into stack 20 where it falls counter-current to the flow of the heated gases into hopper bottom 34. The crushed particles of a size to produce fibers of diameters here referred to, say fibers of 1½-2 micron diameter, will have a fairly definite falling rate such as, say, 7-10 feet per second. The length of the stack between the hopper bottom and supply device 40 is proportioned relatively to the velocity of gas flow up the stack and the temperature of the gases so that the particles will be subjected to the heated gases for a sufficient period to raise them to a temperature approaching that of the gases. This temperature, however, will be below the melting point of the particles. The hot but still solid particles are fed by screw feed 48 through port 32 into furnace 50 where the particles are melted by the relatively higher temperatures present. The enlarged, cross-sectional areas of the cylindrical section and the adjacent end of the conical section of the furnace insures that the flame velocities and the rate of fall of the particles through the furnace are relatively low at this point. The gradual taper and the flattening of the conical section 56 directs the particles along with the flame onto the peripheral surfaces of rotors 64, the flame serving to convey the particles and also to maintain them above their melting temperature until they impinge against and bond to the rotor surfaces. The rotors, suitably about 12" in diameter, as previously stated, are driven at speeds, say, from 4300-5000 R. P. M., although higher speeds may be employed for the production of extremely fine fibers. When the still fluid particles are bonded to the rotors, the particles stretch under the centrifugal forces set up by rotation of the rotors, and are drawn out individually into fibrous form. The fiber formed as described above may be collected by any suitable mechanical or pneumatic equipment (not shown).

In the prior rotor fiberization processes, for example in the processes described in my said copending applications, the use of two or more rotors is essential in that one or more must serve as sub-dividing means to initially divide the molten stream into a storm or cloud of molten particles or droplets which are thrown onto the other rotor or rotors, the latter performing all, or at least a major part of, the fiberizing step. In the instant invention, on the other hand, inasmuch as the molten material is previously subdivided into particle form, each rotor acts individually as a fiberizing means. Consequently, only a single rotor may be used, or if a plurality of rotors are used, they may be rotated so that their upper peripheral surfaces move either toward or away from each other. However, the use of a pair of rotors with their upper peripheral surfaces moving toward each other, as shown in Fig. 1 is preferred, to obtain the desired higher fiber recovery. In order that the molten particles may be drawn out into fibrous form, it is essential that they be bonded to the rotors so that the small molten body making up each particle will be carried by the rotor and a fiber drawn therefrom by the centrifugal forces set up. The preferred direction of rotation of the rotors with their upper surfaces moving toward each other insures such bonding in that, if the force

of the particle in initially striking the rotor is insufficient to cause it to bond, it will immediately be projected by such rotor and at an increased velocity onto the surface of the opposite rotor, the increased velocity of the particle causing it to strike the opposite rotor with sufficient force to adhere to it. The rotation of the rotors in this preferred direction also produces a more tangled mat of fibers desired in most cases.

10 A certain portion of the material striking the rotor surfaces will solidify on them. Such solidified material is usually so refractory that the surfaces of the rotors could not reasonably be kept up to the necessarily high temperature. The use of two rotors, as shown, has the further advantage that this difficulty is eliminated as the rotors are mutually self-cleaning whenever the solidified material becomes excessive in thickness. That is, the solidified material on the opposite rotors will come into contact which causes its dislodgment.

15 In the operation of the apparatus, by far the greater proportion of the molten droplets falling through furnace 50 will retain their individuality and remain free from other droplets or from the walls of the furnace. However, some of the droplets will strike the walls and form a stream which flows down the side walls and drips from the lower edge of the furnace. Where definite control of the fiber size is required for extremely uniform products, this drip may be discarded by drawing it off from the lips in any suitable manner. However, where it is desired to include this material with that to be fiberized, the mouth of the furnace is preferably provided with points 66, as indicated, which tend to break up this stream into a plurality of individual fine streams or drips which become elongated until they contact the rotor surfaces and are drawn out into practically continuous fiber. In order to damp the movement of the particles through the conical section of the furnace and to minimize the impingement on the walls, and also to impart additional heat to the particles, a magnetic flux is preferably set up within the conical section. For this purpose a coil 68 surrounds this section of the furnace, the terminals of the coil being connected to any suitable source of high frequency current, say, a current having a frequency of 1-10 milli-cycles per second.

20 Numerous raw materials may be reduced to fine particle size and fiberized by the instant method. Raw materials of particular merit include plate glass or glass cullet of conventional character, i. e., that having a fluidity which will cause it to flow approximately ½" before solidifying when heated to a temperature of from 2400°-2600° F., basalt, volcanic glass, pyroxene minerals, slag, ash, rock and synthetic mixes which may be specifically prepared for the purpose. These materials will usually require crushing and in this operation the particles are suitably air floated or screened to separate out the predetermined particle size to be employed, the oversized particles being crushed further and the fines being discarded for the present purpose.

25 20 Basalt, when crushed to the proper size to produce fibers of the diameters referred to, contains grains in which two or more minerals are incorporated. These complex mineral grains form complex fiber which has a greater tendency to curl than fiber formed from other of the materials referred to above, and therefore may be referred where heavily curled fiber is desired. However, normally, if the rotors are rotated to

have their upper surfaces moving towards each other, as described above, a sufficient quantity of curled fiber will be made, irrespective of the particular raw material, to give the product good heat-insulating and sound-absorbing properties. A number of the above materials, particularly glass, furnace slag, furnace clinker and basalt, remain solid up to 2000° F. and melt to a ductile fluid condition between 2300° and 2500° F., becoming watery when heated above this temperature. Others of the materials will have different characteristics in these respects. Therefore, it will be understood that the temperatures selected for the operation will be governed by the raw material used.

The preheating operation is designed to raise the temperature of the granulated material close to, but never over, the melting point of the material whereby it is still granular and free-flowing when fed into the melting furnace. The process is thus conducted throughout so that it is not necessary to have working parts such as screw feeds 46 and 48 raised to the melting point of the material which is to be fiberized. The process therefore is especially adapted to fiberizing materials which are extremely refractory and which economically produce very tough and stable fiber. Several of the most desirable and most available materials of those referred to above, including volcanic glass, basalt, fused shale and ash, such materials normally containing combined silica and alumina percentages of over 65%, the balance being mainly lime, iron and magnesia fluxes, and other high silica materials are of the type which produce these stable and tough fibers.

The invention as described above, provides for the production of fibers from numerous raw materials with complete control of the fiber size and uniformity of fiber production, the method of the invention comparing favorably in these respects with the prior individual fiber drawing processes. At the same time the process has the high capacity and economy of the prior multiple fiber forming operations.

Having thus described my invention in rather full detail, it will be understood that these details need not be strictly adhered to but that various changes and modifications may suggest themselves to one skilled in the art, all falling within the scope of the invention as defined by the subjoined claims.

What I claim is:

1. In an apparatus for forming fiber from discrete particles of a fusible raw material, means for subjecting the particles to heated gases to preheat the particles, means for forming a gaseous blast, flame forming means for raising the temperature of the blast above the melting point of the particles, means for discharging the particles from the preheating means into the blast to be conveyed thereby and melted therein, and a fiberizing means in the path of the blast for converting the individual particles into fiber form.

2. In an apparatus for forming fiber of controlled size from discrete particles of controlled size of a fusible raw material, means for subjecting the particles to heated gases to preheat the particles to below their melting temperatures, means for creating a heated gaseous blast, flame forming means for raising the temperature of the blast above the melting point of the particles, means for discharging the particles from the preheating means into the blast to be conveyed thereby and melted therein, and a fiberizing device in the path of said blast, said fiberizing

device including rotors and means for driving the rotors at high speed.

3. In an apparatus for forming fibers from discrete particles of a fusible material comprising a stack, a particle collecting zone in said stack, means for discharging particles into said stack at a point above said zone to permit the particles to fall by gravity to said zone, means for causing a flow of heated gases at a temperature below the melting point of the particles and counter-current to the direction of fall of said particles, means for forming a gaseous blast, means for raising the temperature of the blast above the melting point of the particles, means for discharging the particles from said collecting zone into said blast to be conveyed thereby and melted therein, a fiberizing device and means for directing the gaseous blast and the particles toward said device to deliver the molten particles thereto.

4. In an apparatus for forming fibers from discrete particles of a fusible raw material, a stack, a particle collecting zone in said stack, means in said stack above said collecting zone for discharging particles to permit them to fall by gravity to said collecting zone, means to cause a flow of heated gases at a temperature below the melting point of the particles and counter-current to the direction of fall of said particles, means for forming a heated gaseous blast, flame forming means for raising the temperature of the blast above the melting point of the particles, means for discharging particles from the collecting zone into the blast to be conveyed thereby and melted therein, and means in the path of the blast for converting the individual particles into fibers.

5. In an apparatus for forming fiber from discrete particles of a fusible raw material, a stack, a particle collecting zone in said stack, means in said stack above said collecting zone for discharging particles to permit them to fall by gravity to said collecting zone, means to cause a flow of heated gases at a temperature below the melting point of the particles and counter-current to the direction of fall of said particles, means for forming a heated gaseous blast, flame forming means for raising the temperature of the blast above the melting point of the particles, means for discharging particles from the collecting zone into the blast to be conveyed thereby and melted therein, and means in the path of the blast for converting the individual particles into fibers, said last-named means including rotors adapted to be driven at high speed, and means for driving said rotors.

6. In an apparatus for forming fiber from discrete particles of a fusible raw material comprising heating means, a stack adjacent said heating means, said stack having a particle collecting zone and means in said stack above said collecting zone for discharging particles into said stack to permit said particles to fall by gravity into said collecting zone, means to discharge heated gases at a temperature below the melting point of the particles from said heating means into said stack and to cause them to flow counter-current to the direction of fall of said particles, a melting chamber separate from said stack and having an open mouth, flame forming means in said chamber, means for causing a gaseous blast in said chamber directed toward said open mouth, and means for discharging the particles from said collecting zone into said chamber.

7. In an apparatus for forming fiber from dis-

crete particles of a fusible raw material comprising heating means, a stack adjacent said heating means, said stack having a particle collecting zone and means in said stack remote from said collecting zone for discharging particles into said stack to permit said particles to fall by gravity into said collecting zone, means to discharge heated gases at a temperature below the melting point of the particles from said heating means into said stack and to cause them to flow counter-current to the direction of fall of said particles, a melting chamber separate from said stack and having an open mouth, flame forming means in said chamber, means for causing a gaseous blast in said chamber directed toward said open mouth, means for discharging the particles from said collecting zone into said blast, and fiberizing means opposite said open mouth of the chamber in position to intercept particles carried by said blast from said chamber.

8. In an apparatus for forming fiber from discrete particles of a fusible raw material, means for suspending the particles in a gaseous blast maintained at a temperature above the melting point of the particles, means for directing the particles into a fiberizing zone, and means to establish a magnetic flux within the directing means for damping the particle movement and for maintaining the particles in individualized relationship.

9. In a method of forming fiber from discrete particles of fusible material, the steps comprising subjecting the particles to hot gases in a preheating operation, suspending the pre-heated particles in a gaseous blast maintained

5 at a temperature above the melting point of the particles to melt the particles, conveying the particles in the blast and in discrete relationship to a fiberizing zone, and subjecting the particles in said zone to accelerated movement to draw them out into fibrous form.

10. In an apparatus for forming fiber from a fusible raw material, means for establishing a gaseous blast at a temperature above the melting point of the fusible raw material, means for suspending discrete particles of the fusible raw material in the gaseous blast, means for maintaining the blast at a temperature above the melting point of the particles to melt the particles in said blast, a fiberizing device comprising rotor means, means for rotating the rotor means at high speed, and means for directing the gaseous blast and the discrete particles therein toward said rotor means to deliver the

20 molten particles thereto.

EDWARD R. POWELL.

#### REFERENCES CITED

The following references are of record in the 25 file of this patent:

#### UNITED STATES PATENTS

| Number       | Name     | Date           |
|--------------|----------|----------------|
| Re. 20,828   | Powell   | Aug. 16, 1938  |
| 30 1,769,181 | Jackson  | July 1, 1930   |
| 2,018,478    | Whittier | Oct. 22, 1935  |
| 2,131,599    | Shrum    | Sept. 27, 1938 |
| 2,274,130    | Davis    | Feb. 24, 1942  |
| 2,388,935    | Powell   | Nov. 13, 1945  |
| 35 2,455,908 | Slayter  | Dec. 7, 1948   |